

July 8, 1952

T. D. NIERENBERG

2,602,731

METHOD OF MAKING CIRCUIT PANELS

Filed March 30, 1950

2 SHEETS—SHEET 1



INVENTOR.  
Theodore D. Nierenberg  
BY *Day M. Young*  
his ATTORNEY

July 8, 1952

T. D. NIERENBERG

2,602,731

METHOD OF MAKING CIRCUIT PANELS

Filed March 30, 1950

2 SHEETS—SHEET 2



## UNITED STATES PATENT OFFICE

2,602,731

## METHOD OF MAKING CIRCUIT PANELS

Theodore D. Nierenberg, New York, N. Y., assignor to Etched Products Corporation, Long Island City, N. Y., a corporation of New York

Application March 30, 1950, Serial No. 152,773

12 Claims. (Cl. 41—43)

1

This invention relates to the formation of electric circuit components and, more particularly, to a circuit panel having circuit conductors on one or both surfaces.

One particular use for circuit panels of the type to which the invention is directed, is in automatic business machines, although such panels have many other applications, such as in small radio receivers and the like. As used in automatic business machines, one or both surfaces of a dielectric panel has circuit conductors thereon which may be arranged to cooperate with movable circuit closures or wiper arms of the machine and/or to form complete circuit in cooperation with other electric conductors of the machine. The circuit closures or wipers may, for example, be rotatable or oscillatable to connect with certain conductors on the panel in predetermined sequences or in any set pattern.

As presently constructed, these circuit panels comprise a sheet of dielectric material to which is applied a preformed die-cut sheet of copper or other conductive metal shaped to form the desired arrangement of circuit conductors. The surface of the panel may be suitably recessed, by grinding, routing or the like, to receive the die-cut or otherwise formed copper sheet or copper strips forming the conductors. The resultant circuit panel is not only somewhat expensive in construction but also the circuit bearing surface is not flush, the copper strips usually extending somewhat above the surface of the dielectric panel even when the latter is recessed. As a result, there is considerable resistance to the movement of contacts over the panel in passing, for example, from a dielectric portion to a conductive portion. This causes wear and tear on the contacts and on the circuit conductors, so that frequent replacement of the circuit closures and circuit panels is necessary.

In accordance with the present invention, circuit panels having printed circuits on one or both surfaces are formed in a novel manner whereby the conductive and dielectric portions of the surface are flush and level throughout. Thereby, the aforementioned wear and tear on the circuit closures and conductors is substantially eliminated, resulting in greatly increased life for these elements. In addition, the invention method results in an inexpensively formed circuit panel, having a production cost which is a fraction of that of the prior art panels.

In accordance with the invention, one or both surfaces of a dielectric panel, such as one of a plastic composition material, are coated with a sheet of thin metal foil, such as copper foil, 0.005" or less in thickness. The foil is applied by pressure or pressure combined with the use of a suitable adhesive. Following the foil application, the desired circuit design and arrangement of circuit

2

conductors is imprinted on the foil surfaces by a suitable ink. While the ink is still wet or tacky, the printed surfaces are coated with an acid or etch resist powder. This powder adheres to the ink printed portions, and is easily removed from the non-printed portions.

The article is then etched to remove the foil from the non-printed surface portions, leaving only the desired circuit design comprising conductors coated with ink and the resist powder. The etched out portions are then filled, to a level preferably above the surface of the resist powder, by a suitable dielectric material such as a dielectric paint. This paint may be applied in any desired fashion, certain specific ways being mentioned hereinafter, and is preferably applied in successive layers.

The printed surfaces of the panel are then ground to simultaneously remove some of the insulating material, the etch resist powder, and the ink, all of these materials being removed to the same depth. The resultant panel thus presents smooth, flush surfaces having the foil conductors separated by insulating material in the etched out surface portions. The panel may then be baked to increase the abrasion resistance of the insulator, after which the panel is cut to the desired peripheral contour and formed with any desired holes or apertures.

With the foregoing in mind, it is an object of the present invention to provide an improved, inexpensive circuit panel.

Another object is to provide such a panel having increased life and characterized by flush contact engaging surfaces.

These, and other objects, advantages and novel features of the invention will be apparent from the following description and the accompanying drawings. In the drawings:

Fig. 1 is an elevation view of a completed circuit panel processed in accordance with the invention;

Fig. 2 and Fig. 3 are sectional and elevation views, respectively, of the dielectric base panel with the conductive foil applied thereto;

Fig. 4 is an elevation view of the panel after printing and the application of etch resist powder to the printing;

Figs. 5 through 8 are sectional views, on the line 5—5 of Fig. 4, illustrating the successive steps of the invention method;

Figs. 9 and 10 are elevation views of a completed circuit panel having circuits "printed" on both sides of the dielectric base panel; and

Figs. 11 through 16 are sectional views, on the identical lines 11—11 of Figs. 9 and 10, illustrating successive steps in processing the panel of Figs. 9 and 10.

Referring to Figs. 1 through 8, the invention is illustrated as applied to produce a circuit panel

20 having metal foil conductors such as 25 and 26 thereon. Panel 20 is a circuit panel of the type customarily used in automatic business machines, for example, the several conductors 25 and 26 being suitably connected to operating and/or energizing circuits of the machine.

It will be noted that the several conductors 25 have their inner ends 25a extending in radial relation to a circular aperture 21 in the dielectric base panel 22 on which the conductors are mounted. Correspondingly, the inner end 26a of conductor 26 is arranged as a substantial semi-circle concentric with aperture 21. It will be noted that a circular marginal portion 23 of dielectric panel 22 lies between the inner ends of the conductors and aperture 21.

A rotatable or oscillatable circuit closure or contact member is arranged to engage in aperture 21 and have operative association with conductors 25 and 26, such member forming no part of the present invention and being a standard element of an automatic business machine. It will be understood that circuit panel 20 is merely exemplary of a circuit panel produced according to the present invention, and the particular panel configuration, number of conductors, etc., is in no way a limitation of the invention principles.

Figs. 2 through 8 illustrates steps in forming panel 20 according to the present invention. Referring to Figs. 1 and 2, in the first step of the method as applied to circuit panel 20, a thin sheet of metal foil 30, such as copper foil, for example, is applied to cover one surface of dielectric base panel 22. Foil 30 which may, for example, be 0.005" thick or less, is applied to panel 22 under heavy pressure, or a combination of pressure and adhesive may be used.

As shown in Figs. 4 and 5, the desired circuit design is then imprinted on foil 30 by a suitable adhesive ink as at 31. While the ink is still wet or tacky, the foil covered surface is coated with an acid or etch resist powder as at 32, the powder adhering to the inked portions forming the design and being removed from the non-printed portions of the foil. The foil coated and printed panel is then etched, to remove the non-printed portions of foil 30, as shown in Fig. 6. This leaves the printed and etch resist powder coated portions of the foil forming conductors 25 and 26.

Following the etching step, the portions of the surface of dielectric panel 22 not covered by the conductors 25 and 26 are filled with a suitable electric insulating material 33, such as a dielectric paint, for example. This step is performed while the ink and resist powder coatings remain on conductors 25 and 26, as may be seen from Fig. 7.

Material 33 may be applied in any one of several ways. For example, a dielectric material may be silk-screened onto the etched out portions of the panel, or may be sprayed onto the panel. Alternatively, the paint or the like may be thrown onto the panel and the excess wiped off. The thickness of dielectric material applied to the etched out surfaces is preferably greater than the combined thickness of the foil, ink and resist powder remaining on the printed portions of the surface. This may be effectively accomplished by applying the insulator in successive layers.

The covered surface of the panel is then ground or scraped to remove the resist powder, ink and insulator down to the level of the surface of

conductors 25 and 26. This is effected in a uniform manner so that the surface of the insulator 33 is flush with the surface of conductors 25 and 26 (see Fig. 8), thus providing a smooth, level, flush surface on the circuit side of the panel. Abrasion resistance of the insulator is increased by baking the completed panel, after which the panel is blanked to provide the desired peripheral contour and form aperture 21.

The application of the invention to the formation of a circuit panel 40 having circuits printed on both surfaces is shown in Figs. 9 through 16.

Referring to Figs. 9 and 10, which show opposite surfaces of the completed panel, a dielectric panel 42 is shown as having conductors 45, 46, 47 on one surface and conductors 48 on the opposite surface. Panel 40 has apertures or recesses 39 and 41 in one surface, similar to aperture 21 of panel 20, to receive suitable circuit closures. Also, certain conductors 48 are shown as terminating adjacent small holes 43 to receive wires, eyelets or rivets to complete the circuit connections.

In forming panel 40, sheets 50 and 50' of copper foil, for example, are applied to opposite surfaces of the dielectric base panel 42 by pressure or by pressure and adhesive, as shown in Fig. 11. The designs are then printed on both foil sheets, as indicated at 51, 51', and the sheets coated with resist powder adhering to the inked designs as at 52, 52' (Figs. 12 and 13). The panel is then etched to remove the non-printed and non-coated portions of foils 50, 50', leaving conductors 45, 46 and 47 coated with the ink and the resist powder. The panel now appears in section as shown in Fig. 14.

The etched out portions of the panel then are filled with an insulating material 53, 53' as shown in Fig. 15. The insulator 53, 53' may be applied as previously described, and may be simultaneously applied to both panel surfaces or to one surface at a time. The surfaces are then ground or scraped, either simultaneously or consecutively, to provide surfaces flush with the foil conductors as shown in Fig. 16. The formed panel is then backed to increase the abrasion resistance of the insulator and blanked to shape and to form apertures or recesses 39, 41 and holes 43.

It should be noted that apertures or recesses 39, 41 may be omitted and the corresponding spaces merely act as end stops or bearings for the rotatable or oscillatable circuit closures or wipers.

Although in the embodiments specifically outlined herein, the circuit design was imprinted with a tacky ink to which resist powder was applied, it is within the province of this invention to imprint the foil with a single medium, i. e. an ink or like material which is per se etch resistant, to define the circuit diagram.

The invention provides a circuit panel which has one or more flush surfaces with conductors imprinted thereon. The flush relation of the conductive and dielectric surfaces decreases contact resistance and increases the panel life. Additionally, the panel is much less expensive than those produced by prior art methods.

While specific embodiments of the invention have been shown and described in detail to illustrate the application of the invention principles, it should be understood that the invention may be otherwise embodied without departing from such principles.

What is claimed is:

1. The method of forming an electric circuit

carrying panel which comprises applying conductive sheet material to at least one surface of a panel of dielectric material, removing portions of said sheet material to form a predetermined circuit pattern including individual conductors, applying insulating material to the portions of such surface from which the sheet material has been removed, and finishing the surface of said insulating material flush with the surface of said sheet material.

2. The method of forming an electric circuit carrying panel which comprises applying conductive foil to at least one surface of a panel of dielectric material, removing portions of said foil to form a predetermined circuit pattern including individual conductors, applying insulating material to the portions of such surface from which the foil has been removed, and finishing the surface of said insulating material flush with the surface of said foil.

3. The method of forming an electric circuit carrying panel which comprises applying conductive sheet material to at least one surface of a panel of dielectric material, removing portions of said sheet material to form a predetermined circuit pattern including individual conductors, applying insulating paint to the portions of such surface from which the sheet material has been removed, and finishing the surface of said paint flush with the surface of said sheet material.

4. The method of forming an electric circuit carrying panel which comprises applying conductive foil to at least one surface of a panel of dielectric material, removing portions of said foil to form a predetermined circuit pattern including individual conductors, applying insulating paint to the portions of such surface from which the foil has been removed, and finishing the surface of said paint flush with the surfaces of said foil.

5. The method of forming an electric circuit carrying panel which comprises applying a thin sheet of metal foil to each of the opposed surfaces of a panel of dielectric material, removing portions of said foil sheets to form predetermined circuit patterns, applying insulating paint to the portions of such surfaces from which the foil has been removed, and finishing the surface of said paint flush with the surface of said foil.

6. The method of forming an electric circuit carrying panel which comprises applying conductive foil to at least one surface of a panel of dielectric material, applying an etch resistant layer to said foil in a predetermined circuit pattern, etching the panel to remove foil to form such predetermined circuit pattern, applying insulating material to the portions of such surface from which the foil has been removed to a level at least even with the surface of the resistant layer, and simultaneously removing the etch resistant layer and the insulating material to uncover the foil forming the circuit pattern and bring the surface of the insulating material flush with the foil surface.

7. The method of forming an electric circuit carrying panel which comprises applying conductive foil to at least one surface of a panel of dielectric material, imprinting with ink a predetermined circuit pattern on said foil, before the ink has dried, applying etch resist powder

to the foil, whereby the powder will adhere to the printed pattern foil portions and will not adhere to the non-printed foil portions, etching the panel to remove the non-printed foil portions, applying insulating material to the portions of such surface from which the foil has been removed to a level at least even with the surface of the resist powder, and simultaneously removing the etch resist powder, the ink, and the insulating material to uncover the foil forming the circuit pattern and bring the surface of the insulating material flush with the foil surface.

8. The method of forming an electric circuit carrying panel which comprises applying a thin sheet of metal foil to each of the opposed surfaces of a panel of dielectric material, imprinting with ink predetermined circuit patterns on said foil sheets, before the ink has dried, applying etch resist powder to the foil, whereby the powder will adhere to the printed pattern foil portions and will not adhere to the non-printed foil portions, etching the panel to remove the non-printed foil portions, applying insulating paint to the portions of such surfaces from which the sheet material has been removed to a level at least even with the surface of the resist powder, and with respect to each surface, simultaneously removing the etch resist powder, the ink, and the paint to uncover the foil forming the circuit pattern and bring the surface of the paint flush with the foil surface.

9. The method of forming an electric circuit carrying panel which comprises applying a thin sheet of metal foil to each of the opposed surfaces of a panel of dielectric material, imprinting with ink predetermined circuit patterns on said foil sheets, before the ink has dried, applying etch resist powder to the foil, whereby the powder will adhere to the printed pattern foil portions and will not adhere to the non-printed foil portions, etching the panel to remove the non-printed foil portions, applying insulating paint to the portions of such surfaces from which the sheet material has been removed to a level at least even with the surface of the resist powder, with respect to each surface, simultaneously removing the etch resist powder, the ink, and the paint to uncover the foil forming the circuit pattern and bring the surface of the paint flush with the foil surface, and baking the panel to increase the abrasion resistance of the paint.

10. A method as claimed in claim 7, in which the insulating material is applied by silk screening.

11. A method as claimed in claim 7, in which the insulating material is sprayed on.

12. A method as claimed in claim 7, in which the insulating material is applied in successive layers.

THEODORE D. NIERENBERG.

#### REFERENCES CITED

The following references are of record in the file of this patent:

#### UNITED STATES PATENTS

| Number       | Name          | Date          |
|--------------|---------------|---------------|
| 1,713,951    | Danielson     | May 21, 1928  |
| 2,441,960    | Eisler        | May 25, 1948  |
| 2,498,493    | Hickernell    | Feb. 21, 1950 |
| 70 2,506,604 | Lokker et al. | May 9, 1950   |